

## UNITED STATES PATENT OFFICE

2,472,592

INORGANIC INSULATING COATING FOR  
ELECTRICAL STEEL SHEET AND STRIPGeorge C. Kiefer, Springdale, Pa., assignor to  
Allegheny-Ludlum Steel Corporation, a corpora-  
tion of PennsylvaniaNo Drawing. Application January 9, 1945,  
Serial No. 572,097

5 Claims. (Cl. 148—6.20)

1

This invention relates to the production of a new and improved coating for steel strip or sheet material such as is employed in the make-up of electrical apparatus.

An object of the invention is to provide a coating material which is capable of being spread uniformly over strip or sheet metal, such as for example as silicon steel, and which, when baked, acquires excellent insulating properties but is of such character as not to detrimentally effect the tools and dies employed in fabricating such strip or sheet material.

A further object is to produce an insulating coating for electrical sheet and strip material which is capable of being spread in film-like form and substantially uniformly over the surface of the sheet or strip to be coated and which, in the finished state, has high insulating properties, is insoluble in water and transformer oil and is not detrimentally affected when subjected to temperatures such as are encountered in the use of electrical sheet or strip material or in the preparation of such material for use.

A further object is to produce a coating material for strip or sheet steel which, when applied and baked, provides a protective coating for the covered surface and improves the punching characteristics of the steel so coated.

These and other objects are attained by means of a coating material embodying the characteristics herein set forth and formed from constituents herein set forth or substantial equivalents of the same.

The coating material as formed consists of a mixture of magnesium chromate ( $MgCrO_4$ ), magnesium acetate ( $Mg(C_2H_3O_2)_2$ ) and water ( $H_2O$ ). The preferred mixture includes:

397 pounds magnesium chromate, 7  $H_2O$  (equivalent of 209.2 pounds  $MgCrO_4$ );  
251 pounds magnesium acetate, 4  $H_2O$  (equivalent of 156.7 pounds of  $Mg(C_2H_3O_2)_2$ ), and sufficient water to make 100 gallons of solution.

I have also prepared the coating by mixing 97.1 pounds of magnesium oxide ( $MgO$ ), 154 pounds of chromium trioxide (chromic acid  $CrO_3$ ), 126 pounds of glacial acetic acid  $CH_3COOH$  and sufficient water to make 100 gallons of solution.

Solutions of magnesium chromate (or magnesium oxide and chromic acid) without the addition of magnesium acetate (or acetic acid and magnesium oxide) will produce a coating. Likewise, solutions of magnesium acetate (or acetic

acid and magnesium oxide) without the addition of magnesium chromate (or magnesium oxide and chromic acid) also produces a coating. These coatings, however, are difficult to bake, tend to flake off of the carrying metal after baking and are not satisfactory functionally.

I have also found that, in order to obtain a good adherence of the coating to the metal surface, a proper ratio of chromic acid to acetic acid or magnesium chromate to magnesium acetate must be adhered to. For example, when the weight of magnesium chromate exceeds the weight of magnesium acetate by more than two to one, the resultant coating tends to flake off after baking. On the other hand, when the weight of the magnesium chromate is less than that of the magnesium acetate, the resultant coating is discolored and is slightly brittle when baked. The amount of magnesium chromate by weight should, therefore, exceed that of the magnesium acetate but be less than twice the weight of the acetate.

After the aqueous solution, as above defined, is applied to the surface to be coated, it is baked for a sufficient time to dehydrate and also decompose the salts of the solution. The baking temperature may be as low as 400° F. or as high as 1750° F. I, however, prefer to employ a baking temperature of about 850° F. because a temperature in excess of that tends to evaporate the water in the mixture too rapidly and to occasion blistering and subsequent flaking. The time of baking will vary with the thickness of the coated metal. Baking at 800° F. for two minutes (total exposure), has disclosed itself as sufficient in connection with coated sheets of 0.014" thickness. Thinner sheets will require less time to bake the coated material, and thicker sheets will require more time.

While the above disclosure defines the preferred solution and the preferred procedure for making the same, a suitable coating material can be made by the above enumerated constituents within the limits defined as follows:

45 85.75 to 121.5 pounds magnesium oxide ( $MgO$ )  
124.5 to 180 pounds chromium trioxide (chromic acid)  $CrO_3$   
105 to 148 pounds glacial acetic acid ( $C_2H_3O_2$ ),  
50 and sufficient water to make 100 gallons; or  
330 to 473 pounds magnesium chromate, 7  $H_2O$  (equivalent of 175 to 250 pounds  $MgCrO_4$ )  
187 to 263 pounds magnesium acetate, 4  $H_2O$  (equivalent of 125 to 175 pounds  $Mg(C_2H_3O_2)_2$ ),  
55 and sufficient water to make 100 gallons.

These solutions applied on metal surfaces and baked, as defined herein, result in coatings which are insoluble in water or oil, possess excellent insulating properties and are not destroyed or detrimentally affected when subjected to temperatures as high as 1750° F. As a matter of fact, coatings subjected to such temperatures for an appreciable period (about 30 minutes) have disclosed increased insulating values.

While the constituents of the coating solution are soluble in water as above disclosed, the baking temperature not only dehydrates the solution defined but it also decomposes the constituents thereof and the resulting coating is insoluble in water and oil. The coating, while of complex chemical composition, undoubtedly includes magnesium oxide, chromium oxide and some iron oxide. The iron oxide possibly results from the fact that some oxygen is released from the magnesium salts during their decomposition and, while in a more or less nascent state, forms an oxide with the metal to which the coating is applied with the result that such metal also provides an oxide or other constituent of the coating.

The procedure herein set forth, as an embodiment of my invention, may be briefly stated as coating electrical strip or sheet material with a thin film of an aqueous solution containing magnesium chromate and magnesium acetate (no matter how formed) and in which the amount of chromate by weight is preferably greater than that of the acetate but less than twice the weight of the acetate, and then subjecting the material so coated to sufficient heat to dehydrate such film and to decompose the magnesium compounds constituting constituents thereof. The baked or dehydrated coating not only provides an insulating film which is highly effective when applied to electrical sheet or strip material used in the fabrication of electrical apparatus but, it also provides a protective coating which facilitates the punching or shearing of metallic sheet or strip material whether or not the same is formed from electrical sheet. It, therefore, is apparent that the dehydrated coating does not have a detrimental effect on the tools and dies employed in the fabrication of such material. I have also found that the dehydrated coating gives good results as a protective coating for steel sheet or strip material that has either been parkerized, bonderized, or treated with some similar phosphate coating.

While coatings embodying my invention may be varied as to their constituents, within the limits above defined, all such coatings, nevertheless, involve mixtures of inorganic materials such as defined and produces a coating for electrical sheet and strip material which has many times the resistance value of other commercial coatings now employed for such materials. It will be understood by those skilled in the art that some additional materials may be added as constituents to coatings, such as are above defined, without departing from the spirit and scope of my invention as defined by the appended claims and that the temperature range for baking the same may be widely varied within the limits above defined.

What I claim is:

1. A method of forming an insulating coating on electrical steel in sheet or strip form, which consists in spreading an aqueous solution over the surface of such steel to form a film-like coating thereon, which solution consists essentially of

magnesium chromate and magnesium acetate in which the chromate exceeds the acetate by weight in an amount less than twice the weight thereof, then in subjecting the coated steel to sufficient heat at a temperature of about 850° F. to dehydrate such coating and decompose the magnesium salts contained therein.

2. A method of forming an insulating coating on silicon steel in sheet or strip form, which consists in coating the surface of such steel with an aqueous solution the solutes therein consisting essentially of magnesium chromate and magnesium acetate in the proportions of about two hundred parts by weight of chromate and one hundred and fifty parts by weight of acetate and then subjecting the coated steel to sufficient heat within the range of from about 400° F. to 1750° F. to dehydrate such film and decompose such salts.

3. A method of forming an insulating coating on silicon steel in strip or sheet form, which consists in coating at least a surface of such steel with an aqueous solution the solutes therein consisting essentially of magnesium chromate and magnesium acetate in which the chromate exceeds the acetate by weight but in an amount less than twice the weight thereof, then subjecting the material so coated to sufficient heat within the temperature range of from 400° F. to about 1750° F. to dehydrate such coating and to decompose the magnesium salts contained therein.

4. A method of forming an insulating coating on silicon steel in sheet or strip form, which consists in coating the surface of such steel with an aqueous solution of magnesium chromate (7H<sub>2</sub>O) and magnesium acetate (4H<sub>2</sub>O) in the proportion of from about 330 to about 473 pounds of magnesium chromate and from about 187 to about 263 pounds of magnesium acetate in approximately sufficient water to make 100 gallons of solution with the amount of chromate in excess of the acetate by weight but in an amount less than twice the weight thereof, then subjecting the material so coated to heat within the range of from about 400° F. to 1750° F. for a sufficient period to dehydrate such coating and decompose said magnesium salts.

5. An electrical steel sheet coated with a firmly adherent coating insoluble in oil and water and including as essential constituents thereof magnesium oxide and chromium oxide, resulting from the dehydration and decomposition by heat within the range of from 400° F. to 1750° F., of an aqueous solution while spread over the surface of such sheet, the solutes thereof consisting essentially of magnesium chromate and magnesium acetate in which the chromate exceeds the acetate by weight but in an amount of less than twice the weight of the acetate.

GEORGE C. KIEFER.

#### REFERENCES CITED

The following references are of record in the file of this patent:

#### UNITED STATES PATENTS

| Number    | Name                   | Date           |
|-----------|------------------------|----------------|
| 589,221   | Placet -----           | Aug. 31, 1897  |
| 2,144,425 | Cook -----             | Jan. 17, 1939  |
| 2,210,850 | Curtin -----           | Aug. 6, 1940   |
| 2,224,245 | Allen -----            | Dec. 10, 1940  |
| 2,308,070 | Frey -----             | Jan. 12, 1943  |
| 2,354,123 | Horstman et al. -----  | July 18, 1944  |
| 2,385,332 | Carpenter et al. ----- | Sept. 25, 1945 |

**Certificate of Correction**

Patent No. 2,472,592.

June 7, 1949.

**GEORGE C. KIEFER**

It is hereby certified that errors appear in the printed specification of the above numbered patent requiring correction as follows:

Column 4, lines 39 and 40, claim 4, strike out the word "approximately" and insert the same after "make" in line 40;

and that the said Letters Patent should be read with these corrections therein that the same may conform to the record of the case in the Patent Office.

Signed and sealed this 1st day of November, A. D. 1949.

[~~SEAL~~]

**THOMAS F. MURPHY,**  
*Assistant Commissioner of Patents.*